

## United States Patent Office

2,956,898

Patented Oct. 18, 1960

1

2,956,898

## BRIGHTENING AGENTS

Fritz Fleck, Bottmingen/Basel, Switzerland, assignor to Sandoz Ltd., Basel, Switzerland

No Drawing. Filed Sept. 3, 1958, Ser. No. 758,678

Claims priority, application Switzerland Sept. 20, 1957

11 Claims. (Cl. 117—33.5)

The present invention relates to the improvement of the "white content" of organic materials, more especially fibrous materials, such as textile fibers and paper fibers, and products (fabrics, sheets, foils, etc.) made therefrom, and is characterized in that the said materials are treated with a dilute aqueous solution of a blue-fluorescing compound of the formula



wherein X stands for a halogen atom, Y stands for the radical of a secondary mono-hydroxyalkylamine which contains 3 to 5 carbon atoms, and M stands for H or an alkali metal cation.

According to the present invention, the compounds of Formula I are valuable brightening agents for textile fibers, paper and the like and are distinguished from comparable known brightening agents by superior fastness properties, particularly by especially good fastness to light and fastness to washing.

The brighteners I of the present invention can be prepared e.g. by reacting two mols of cyanuric halide (e.g. cyanuric chloride) with one mol of 4,4'-diaminostilbene-2,2'-disulfonic acid or alkali metal salt thereof and with two mols of a mono-hydroxyalkylamine which contains 3 to 5 carbon atoms.

Illustrative of the radicals Y derived from the aforesaid secondary mono-hydroxyalkylamines are, for example, N-methyl-N-β-hydroxyethylamine, N-ethyl-N-β-hydroxyethylamine, N-isopropyl-N-β-hydroxyethylamine.

The action of the brighteners is based upon their capacity to convert invisible ultraviolet light into visible blue to violet fluorescent light.

The compounds employed according to the present invention produce especially good brightening effects on polyamide fibers, such as nylon, Perlon, Grilon, wool, silk, etc., but good brightening effects are also realized on cellulose fibers, such as cotton, staple rayon, viscose, paper, etc.

For the polyamide type of fiber, the brightening is produced either in an exhausting (or drawing-on) process from a neutral to weakly acid bath, primarily at temperatures between 50 and 100° C. or on the foulard with subsequent heat treatment, e.g. steaming at 100 to 120° C. For the cellulosic fiber, use is preferably made of an exhausting process from a neutral to weakly alkaline bath which contains a salt, such as Glauber's salt, at temperatures between 20 and 80° C.

The brightening according to the present invention may be carried out per se, i.e. as an independent process, or in combination with other processing treatment, such e.g. as a finishing process, washing, chemical bleaching, softening, etc.

The brighteners I are most advantageously employed in concentrations of 0.02 to 0.5% by weight, relative to the weight of the goods being treated.

As previously indicated, the obtained brightening effects are especially fast to light and to washing.

In the optical brightening of polyamide fibers, it is particularly important that the brightened products be

2

able to withstand the thermo-fixing process which usually takes place at the end of the finishing treatments. This requisite fastness to temperature is possessed in a very high measure by the compounds I employed according to the present invention.

Another advantage possessed by the brighteners I, in comparison to the comparable prior brighteners, is that they yield more brilliant brightening effects when employed in increasing concentration.

The compounds I contain in the molecule thereof two reactive halogen (chlorine) atoms which can react with water, amines, phenolates, alcoholates and alkalies at temperatures above 60 to 70° to yield new substances of generally enhanced fluorescence but with somewhat

slightly lower fastness properties. It was therefore to be assumed that when using these compounds on the fiber, a temperature of about 50° C. should not be exceeded.

However, the brighteners I do not yield a sufficient brightening effect on the polyamide type of fiber, when employed at temperatures between 20 and 50° C. It was therefore most unexpected and surprising that when used at increased temperature between 50 and 100° C., not only was there an enhanced brightening effect but also—and this, in particular, was wholly unforeseeable—a considerable and significant increase in fastness properties, such as fastness to light and fastness to washing, of the resultant brighteners.

This unexpected stability makes it possible to employ the compounds I as white-toners in textile finishing. This represents an important step forward in this field.

The following illustrative examples set forth presently-preferred exemplary embodiments of the invention. In the said examples, the parts and percentages are by weight. Temperatures are in degrees centigrade.

## Example 1

25 milligrams per liter of sodium 4,4'-bis-(2-(methyl-β-hydroxyethylamino)-4-chloro-1,3,5-triazyl-(6)-amino)-stilbene-2,2'-disulfone are added to an aqueous 40 peracetic acid-bleaching bath which contains 2 grams per liter of peracetic acid of 30% strength, after which nylon piece goods are bleached in the said bath in a goods-to-liquor ratio of 1:40 by weight for 30 minutes at 70° and for 15 minutes at 80°. The nylon which may be undyed 45 nylon filament fabric (polyamide of the sebacic acid-hexamethylene diamine polycondensate type; has a whiter appearance—after being rinsed and dried—than a specimen of the same material similarly treated but in the absence of the brightener.

50 The same whitening effect is obtained if the same material is first treated with the said brightener in the presence of 0.6 gram per liter of aqueous treating bath, and only thereafter treated in the peracetic acid-bleaching bath of the afore-indicated composition.

## Example 2

55 Undyed wool skeins, pre-bleached with hydrogen peroxide, are moved about for 20 minutes at 75° in a goods-to-liquor ratio of 1:40 by weight in an aqueous bath 60 which contains 50 milligrams per liter of 4,4'-bis-(2-β-hydroxydiethylamino-4-chloro-1,3,5-triazyl-(6)-amino)-stilbene-2,2'-disulfonic acid and is at a pH of 4 (adjusted with the aid of acetic acid). The material is then rinsed and dried. The wool is distinctly brightened.

## Example 3

65 Bleached sulfite cellulose is ground for 20 minutes in the hollander at a pulp density of 1:40 in the presence of 0.05% of sodium 4,4'-bis-(2-isopropyl-β-hydroxyethylamino-4-chloro-1,3,5-triazyl-(6)-amino)-stilbene-2,2'-disulfone and, after diluting the mass with water to a pulp density of 1:200, it is worked up into

the form of paper. The paper has a distinctly brighter appearance than an analogous paper prepared without the brightener.

After grinding or beating thereof, the paper mass can be sized with 2% of rosin and 3% of aluminum sulfate. The resultant paper, otherwise treated with the brightener as described in the preceding paragraph, has the same white content as the first-described paper product.

*Example 4*

Nylon piece goods, such as is employed in Example 1, is washed for 20 minutes at 80-90° in a goods-to-liquor ratio of 1:20 by weight in an aqueous washing bath which contains, per liter, 1 gram of octylphenyldecaglycolether, 10 milligrams of the brightener employed in Example 1 and 0.1 gram of acetic acid. The washed material is then rinsed and dried. The obtained nylon is of distinctly brightened aspect.

A similar effect is obtained when, in the preceding paragraph, the brightener of Example 1 is replaced by the same quantity of one of the brighteners used in Examples 2 and 3.

The octylphenyldecaglycolether may, with like success, be replaced by any wash-active polyglycolether or by an acid-resistant anion-active washing agent such for example as sodium oleoylmethyltauride.

Having thus disclosed the invention what is claimed is:

1. A method of enhancing the white content of organic material, which comprises treating the said material with a dilute aqueous solution of a blue-fluorescing compound of the formula



wherein X stands for a halogen atom and M stands for a cation including hydrogen.

2. A method of enhancing the white content of textile fibrous material, which comprises treating the said materials with a dilute aqueous solution of a blue-fluorescing compound of the formula



wherein X stands for a halogen atom and M stands for a cation including hydrogen.

3. A method of enhancing the white content of paper, which comprises treating the said material with a dilute aqueous solution of a blue-fluorescing compound of the formula



wherein X stands for a halogen atom and M stands for a cation including hydrogen.

4. A method of enhancing the white content of a polyamide, which comprises treating the said material

with a dilute aqueous solution of a blue-fluorescing compound of the formula



wherein X stands for a halogen atom and M stands for a cation including hydrogen.

5. A method of enhancing the white content of cellulose-containing organic material, which comprises treating the said material with a dilute aqueous solution of a blue-fluorescing compound of the formula



wherein X stands for a halogen atom and M stands for a cation including hydrogen.

6. A method of enhancing the white content of organic material, which comprises treating the said material with a dilute aqueous solution of a blue-fluorescing compound of the formula



wherein X stands for a halogen atom and M stands for a cation including hydrogen, in a treating bath at a temperature between 50 and 100° C.

7. A method of enhancing the white content of organic material, which comprises treating the said material with a dilute aqueous solution of a blue-fluorescing compound of the formula



wherein X stands for a halogen atom and M stands for a cation including hydrogen, on the foulard, followed by steaming at a temperature of 100 to 120° C.

8. A method of enhancing the white content of organic material, which comprises treating the said material with a dilute aqueous solution of a blue-fluorescing compound of the formula



wherein X stands for a halogen atom and M stands for a cation including hydrogen, said compound being present in an amount of about 0.02 to about 0.5% by weight relative to the weight of the material being treated.

9. A method of enhancing the white content of organic material, which comprises treating said material with a dilute aqueous solution of sodium 4,4'-bis-2-(methyl- $\beta$ -hydroxyethylamino)-4-chloro-1,3,5-triazyl-(6)-amino)-stilbene-2,2'-disulfonate.

10. A method of enhancing the white content of organic material, which comprises treating said material with a dilute aqueous solution of 4,4'-bis-(2- $\beta$ -hydroxy-diethylamino-4-chloro-1,3,5-triazyl - (6) - amino)-stilbene-2,2'-disulfonic acid.

11. A method of enhancing the white content of organic material, which comprises treating said material with a dilute aqueous solution of sodium 4,4'-bis-(2-isopropyl- $\beta$ -hydroxyethylamino - 4 - chloro-1,3,5-triazyl-(6)-amino)-stilbene-2,2'-disulfonate.

## References Cited in the file of this patent

## UNITED STATES PATENTS

|    |           |                 |                |
|----|-----------|-----------------|----------------|
| 10 | 2,778,827 | Ackermann ----- | Jan. 22, 1957  |
|    | 2,805,999 | Ackermann ----- | Sept. 10, 1957 |

## FOREIGN PATENTS

|    |         |                     |               |
|----|---------|---------------------|---------------|
| 15 | 528,445 | Canada -----        | July 31, 1956 |
|    | 715,239 | Great Britain ----- | Sept. 8, 1954 |

UNITED STATES PATENT OFFICE  
CERTIFICATION OF CORRECTION

Patent No. 2,956,898

October 18, 1960

Fritz Fleck

It is hereby certified that error appears in the above numbered patent requiring correction and that the said Letters Patent should read as corrected below.

Column 2, line 46, for "polycondensate type; has" read  
-- polycondensate type; "Nylon 610"), has --.

Signed and sealed this 1st day of August 1961.

(SEAL)

Attest:

ERNEST W. SWIDER  
Attesting Officer

DAVID L. LADD  
Commissioner of Patents